

# UNITED STATES PATENT OFFICE.

HANS REBS, OF DUSSELDORF, GERMANY.

## DRYING-OIL AND PROCESS OF MAKING SAME.

1,201,625.

Specification of Letters Patent. Patented Oct. 17, 1916.

No Drawing.

Application filed June 24, 1916. Serial No. 105,687.

To all whom it may concern:

Be it known that I, HANS REBS, citizen of Germany, residing at Dusseldorf, Germany, have invented certain new and useful Improvements in Drying-Oil and Process of Making Same; and I do hereby declare the following to be a full, clear, and exact description of the invention, such as will enable others skilled in the art to which it applies to make and use the same.

When ordinary non-volatile mineral oils of high boiling point are mixed with vegetable oils which dry more readily, such as linseed oil, the time necessary for drying is considerably lengthened, even when small quantities only of mineral oil are present. Although the thin film then formed may feel dry, the layer is not homogeneous and the difference between the dry linoxyn and the still wet mineral oil is easily distinguished. It is possible to separate the mineral oil from such mixture by extraction or centrifugal action. In mixtures of rapidly drying vegetable oils, such as varnish, with mineral oils, the latter readily separate and accumulate on the surface of the coating, forming a damp greasy layer on the same. In all these cases the mineral oil is only apparently dry and thus the mixture of a dry oil or varnish with mineral oil is considered to deteriorate the quality of the former very considerably.

The object of the present invention is not only to avoid the above named disadvantages, but also to render the mineral oil actually capable of drying. I attain this object by mixing mineral oils perfectly free from paraffin, and having a freezing point of about 30 degrees C. and a boiling point of preferably 300 degrees C. to 310 degrees C., either in hot or cold condition, with a vegetable oil or vegetable oil mixture, thickened either by continuous boiling, by oxidation, or by vulcanization, and then adding drying substances to produce varnish.

Thus, as an example, 100 parts by weight of linseed oil and 50 parts by weight of wood oil are thickened by continuous boiling and, on the completion of this process, 500-700 parts by weight of mineral oil free from paraffin and having a boiling point of 300°-310° C. are added. Or 100 parts by weight of linseed oil and 50 parts by weight of wood oil are thickened at a corresponding temperature by feeding in air or oxygen, and on the completion of the

process are mixed with 500-700 parts by weight of a mineral oil free from paraffin. Or again, 100 parts by weight of linseed oil and 50 parts of wood oil are vulcanized at a corresponding temperature with 2-3% of flower of sulfur or a corresponding quantity of chlorid of sulfur and on completion of the process, from 500-700 parts by weight of mineral oil free of paraffin are added. Owing to the high boiling point of the mineral oil, it is possible to carry out the process described of thickening the oil, in the presence of the mineral oil and in this case products richer in quality are obtained. Drying substances are added according to requirements, i. e. according to the drying properties required of the varnish to be produced from the mineral oil rendered driable.

The non-volatile mineral oils of high boiling point hitherto employed for merely mixing with varnishes always contained a large amount of paraffin and were consequently not proof against the cold. It is an important feature of the present invention that mineral oils be employed, which are not only absolutely proof against the cold but also perfectly free from paraffin. From 10 to 15% of paraffin oil thickened in the above described manner to a kneadable degree will be sufficient to render a perfectly paraffin-free mineral oil capable of being dried to a homogeneous elastic degree within a normal period of time, which period may be reduced to the shortest one of about 7 hours by adding suitable drying agents. In every case the coating film obtained will be dry to the touch, and form a homogeneous whole, the individual constituent parts of which cannot be mechanically separated. This constitutes an extraordinary technical effect.

A varnish prepared in the above described manner may consist of from 80 to 90% of mineral oil, and will not differ from a pure oil varnish in its technical qualities for painting and varnishing purposes, while mixtures of linseed oil varnish, with only 5% of the ordinary mineral oil are objectionable.

It has been found that a varnish made from this mineral oil thus rendered capable of being dried possesses the same quality of binding colors and is also weather proof, to a degree equal to pure oil varnish, and is particularly suitable for the production

of rust-proof coatings. Mineral oil, thus rendered capable of drying is particularly well suited for making all kinds of varnishes from resins and copals, a purpose for which it has hitherto been impossible to employ mineral oils.

I am aware that the obtaining of mineral oils of high boiling point and entirely free from paraffin is known; the separation of 10 paraffin from mineral oils containing the same is based on the fact that paraffin is rendered solid on cooling the mineral oil and is eliminated by being pressed out. The greater the degree of cold employed, the 15 more easy and more perfect will be the separation of the paraffin.

I claim as my invention:—

1. A composition of matter, comprising an admixture of thickened vegetable oil 20 and a mineral oil having a boiling point of approximately 300 degrees C. and being free of paraffin.

2. A composition of matter, comprising an admixture of thickened vegetable oil

with a preponderating quantity of a mineral oil having a boiling point of approximately 300 degrees C. and being free of 25 paraffin.

3. The herein described process of producing an oil composition, which consists 30 in admixing thickened vegetable oil with mineral oil having a boiling point of approximately 300 degrees C. and being free of paraffin.

4. The herein described process of producing an oil composition, which consists 35 in admixing vegetable oil with mineral oil having a boiling point of approximately 300 degrees C. and being free of paraffin, and thickening such vegetable oil in the 40 presence of the mineral oil.

In testimony whereof I hereunto affix my signature in the presence of two witnesses.

HANS REBS. [L.S.]

Witnesses:

ALBERT NUFER,  
HELEN NUFER.